

## UNITED STATES PATENT OFFICE

FRANK WALTER STEERE, OF SCARSDALE, NEW YORK, ASSIGNOR TO THE BARRETT COMPANY, OF NEW YORK, N. Y., A CORPORATION OF NEW JERSEY

## METHOD OF PRODUCING COKE

No Drawing.

Application filed February 1, 1928. Serial No. 251,233.

This invention relates to improvements in the operation of by-product coke oven plants whereby the maximum yield of merchantable coke can be produced, together with other valuable by-products.

In the operation of coke oven plants the coke is delivered from the ovens in an incandescent state and it is necessary to cool it as quickly as possible to avoid combustion with consequent loss of coke. This cooling is commonly effected by quenching with water. The coke, after cooling, is classified into the various sizes required by the trade. It must in some cases be crushed to eliminate larger lumps and to provide higher yields of definite sized pieces. The grading of the coke into different sizes is accomplished by a screening operation. During the quenching, screening and handling of the coke some of it is broken up or degraded into pieces too small to be marketed as commercial coke products. Such coke is commonly known as breeze. When crushing is resorted to the percentage of breeze will in general be higher than when the coke is not crushed. In general, all coke which will pass through a three-quarter inch mesh screen is included as coke breeze, although in some cases only the coke particles passing through a half inch mesh screen are so designated. The amount of coke breeze passing through a three-quarter inch mesh screen will ordinarily amount to around four to six percent of the coke produced but may in some cases run to a higher amount, around ten percent or higher.

Coke breeze in general finds no market and it is commonly disposed of by burning it as fuel, for which purpose its value is far below that of merchantable coke.

It has been proposed to convert coke breeze into marketable fuel by briquetting it with various binders, but this requires the grinding of the coke breeze to produce uniform sizes of particles suitable for briquetting, and the subsequent forming of the ground coke breeze into briquettes by a briquetting operation. This grinding of the coke breeze, in addition to its expense, is objectionable because of the wear and tear on the grinding equipment, with the result that the grinding

and briquetting of coke breeze has been carried out only to a limited extent.

Coke breeze has also been added to the coal charged into coke ovens (see United States patent to Graul, No. 1,308,754). The coal charged to coke ovens is commonly ground and in many cases is pulverized before it is charged to the ovens in order that it may be in the form of fine particles when charged; and the coke breeze employed has similarly been employed in the form of fine particles charged with the finely divided coal.

Coke breeze can be crushed or ground and converted into fine particles similar to those of the coal charged to the coke ovens, but the wear and tear on the crushing apparatus is excessive, and the cost and difficulty of grinding or crushing the coke breeze to produce uniformly small particles out-weighs to a large extent the advantages resulting from returning the coke breeze to the coke ovens.

The present invention provides an improved process of operation of by-product coke oven plants whereby the coke breeze can be advantageously utilized for the production of merchantable coke, and whereby only gas, merchantable coke and by-products need be produced at a coke oven plant.

According to the present invention the coke breeze, without crushing and containing not only the finer particles but also the larger pieces which pass through a screen of around one-half to three-quarters inch mesh during the screening operation, is added to the coal charged to the oven, and the admixed coke breeze and coal are subjected to coking. By operating in this way, all of the coke produced can be sold as merchantable coke, that returned to the coke ovens as breeze being combined with the coal on coking to form merchantable coke and the coke breeze therefrom being returned in a similar way in further operation.

The coal employed in the coke oven operation, where the coke breeze is added to and admixed therewith, should be a coal having sufficient coking properties and constituents to cause the coke breeze to become blended therewith. Domestic coke is commonly produced from coal rich in volatile and coking

constituents in order to produce a larger amount of merchantable gas from the coking and gas making operation. With rich gas making coal the coke breeze will be blended or incorporated therewith on coking so that the particles of the coke breeze will largely or entirely lose their identity in the resulting coke produced.

With some coals it is advantageous to employ pitch by adding it to the charge of coal and coke breeze so that the admixed charge which is subjected to coking will contain coke breeze, pitch and coal. This enables any excess production of pitch to be converted into merchantable coke, gas and tar simultaneously with the coking of the coal, and gives a composite product containing pitch coke as well as coke breeze combined with coal coke.

When pitch is employed in the present process, it can be readily produced by the distillation of the tar separated from the coke oven gases in the by-product recovery system of the coke oven plant. This by-product tar, on distillation, yields merchantable oils and a pitch residue. By returning the pitch residue to the coke ovens in admixture with coke breeze and coal it is subjected to destructive distillation in the coke ovens and converted in part into pitch coke and in part into gas and tar. By utilizing all of the tar produced at the coke oven plant in this way, the plant can be operated so that only salable products, namely, merchantable coke, gas, coal tar distillates and such products as ammonia and/or light oil, are produced at the coke oven plant.

The distillation of the tar to produce therefrom salable oils can be carried out in ordinary tar stills, but is more advantageously carried out by distillation of the tar by direct contact with hot coke oven gases. The gases employed for the distillation may be freed from heavy tar and pitch constituents by scrubbing with hot pitch or by cleaning with an electrical precipitator. Clean salable coal tar oils may be recovered when the gases carrying the oil vapors are subsequently cooled to condense the oils. The distillation of the tar can be carried to a point such that pitch of high melting point is produced, with a high yield of marketable oils. The pitch may, for example, have a melting point around 300° F., or around 400° F., or in some cases even higher. The total pitch produced from the tar can be returned to the coke ovens along with the total amount of coke breeze. Additional pitch may, however, be employed such as may be produced by the distillation at the coke oven plant of tar from outside sources.

In mixing the coal and coke breeze, or coal, coke breeze and pitch, before charging the mixture to the coke ovens, the mixing operation is conducted without passing the coke breeze through the pulverizer for the coal. The coke breeze may be supplied continuously

in regulated amount along with the coal and pitch to the mixing bin.

The coke breeze can advantageously first be admixed with the pitch before the admixed coke breeze and pitch are mixed with the coal. A particularly advantageous form of preliminary admixture of the coke breeze and pitch is by adding the pitch in a hot molten and thinly fluid state to the coke breeze and permitting it to solidify in contact therewith. This method of admixture coats the coke breeze with the pitch and insures that the pitch will be in close proximity to the coke breeze during the coking operation. The molten pitch both during the mixing operation and during the subsequent coking operation in the coke oven penetrates and coats the larger pieces of coke breeze, and, during the coking operation, the coking of the pitch produces pitch coke within the pores of the coke particles and on the surface thereof, thus assisting in binding the coke breeze particles to the coke produced from the coal.

The proportions of coke breeze and pitch blended with the coal charged to the coke ovens can be varied. In some cases the amount of coke breeze produced will be only around five or six percent or less of the total coke produced, while in other cases it may be as high as 10% or more of the coke produced. The amount of pitch employed may be around one percent or somewhat less of the coke oven charge or it may be increased to several percent, e. g., ten to fifteen percent, particularly with high melting point pitch, e. g., around 400° F., melting point.

When pitch is added to the charge it serves as a coking constituent for the breeze, supplementing the coking constituent of the coal, that is, the pitch serves as a flux or binder for the coke breeze particles and aids in binding them to the coal coke produced and tends to give a more uniform structure, particularly where the pitch is admixed and combined with the coke breeze before they are admixed with the coal of the charge.

The coking of the composite charge can be carried out in the usual way. During the coking operation the coke breeze will remain practically inert, but the pitch will liquefy and become coked to form pitch coke and the coal will also be coked in admixture therewith. The composite coke produced will contain the coke breeze, including pieces of coke breeze up to, for example, one-half or three-quarter inch size, distributed throughout the coke product, which will also contain pitch coke produced from the pitch charged to the oven.

In the operation of coke ovens containing e. g., around five or ten percent of coke breeze and containing e. g., one to five per cent of pitch of 300° F. or 400° F. melting point, the tar produced per ton of coke may be somewhat less than ordinarily produced from coal.

to which no coke breeze is added. The yield of tar per ton of coal coked will, however, not be changed materially. The coking of the pitch will result in destructive distillation and the driving off of part of the pitch as gas and as oil or tar constituents which will be collected with the gas and tar from the distillation of the coal. The composite tar so produced can be subjected to distillation for the production of marketable distillate oils, such as creosote oils, and to produce additional pitch for use in the further carrying out of the process.

This method of operation utilizes all of the coke breeze produced at the coke oven plant and utilizes all of the tar produced at the coke oven plant, with the production of coke, distillate oils and gas as the only primary products, together with such by-products as ammonia and light oils. A coke oven plant operated in this way produces only merchantable products and a greatly increased yield of marketable coke from the coal employed. The fuel for the boilers or for other purposes now commonly provided by burning the coke breeze can be supplied from other sources such, e. g., as water-gas machines or gas producers.

When pitch is not added to the coke oven charge, the coking constituents of the coal will be relied upon to bind the particles of coke breeze to the pitch coke produced and, as above stated, with some coals rich in coking or volatile constituents, considerable coke breeze can be added without crushing and incorporated in the coal coke produced.

The present invention is of particular value for the production of domestic coke. Whereas in metallurgical coke operations, large pieces of uniform structure are desirable, this is not the case when the coke is being made for domestic use, where large pieces are a disadvantage in that they have to be crushed. Any lack of uniformity of the coke produced by the present invention is therefore unobjectionable in domestic coke, and such weakening of the coke structure as may be brought about by the presence therein of the particles of coke breeze of varying sizes up to around e. g., one-half or three-quarter inch size is of advantage in reducing the amount of crushing required to convert the coke into domestic sizes.

The present invention is not limited to the use of the smaller coke particles commonly included as coke breeze, since pieces of coke somewhat larger than those ordinarily included in coke breeze can be returned to the coke oven charge in a similar way. Accordingly, where the market price of the smaller sizes of coke is sufficiently below that of the larger sizes, the smaller sizes can be returned to the coke oven in admixture with the coal, or with coal and pitch, and thereby incorporated in the coke charge produced. The

larger sizes of coke from such coke charge can then be marketed at the higher prices, and the smaller low price charges of coke again returned to the coke ovens in further operations. In general, however, only the smaller sizes of coke, such as are commonly classified as coke breeze, and which do not have a ready market as domestic coke, will be returned to the coke oven charge, in order that they may be converted into a product merchantable as domestic coke.

I claim:—

The method of producing coke which comprises admixing coke breeze and hot liquid pitch, cooling the mixture to solidify the pitch in admixture with the coke breeze, adding the resulting coke breeze and pitch to coal charged to a coke oven, and coking the resulting charge.

In testimony whereof I affix my signature.

FRANK WALTER STEERE.

90

95

100

105

110

115

120

125

130